

## UNITED STATES PATENT OFFICE

2,378,793

## STABILIZATION OF ORGANO-METALLIC AGENTS

Harry W. Rudel, Roselle Park, N. J., assignor to  
Standard Oil Development Company, a corpora-  
tion of Delaware

No Drawing. Application March 26, 1942,  
Serial No. 436,329

5 Claims. (Cl. 44—69)

This invention deals with the protection of an organo-metallic agent, particularly with the protection of tetraethyl lead which is used in refined gasoline motor fuels as an anti-knock agent.

Thus far, tetraethyl lead has proved to be the most practical organo-metallic anti-knock additive. The gasoline fuels in which this additive is used have to be well refined to remove sulfur-containing compounds which depress its effectiveness, but furthermore, it has been found desirable to overcome the tendency of this agent to become deteriorated by the action of light.

Investigations have shown that light breaks down tetraethyl lead and thereby forms a precipitate of lead compounds even if the tetraethyl lead is present in refined fuels which are stable toward oxidation or contain effective anti-oxidants. For example, to obtain a true measure of the storage stability of aviation gasolines containing tetraethyl lead, it was found essential to protect the leaded gasoline samples from direct or diffused light before they are subjected to conventional accelerated gum tests. The deteriorating effect of light manifests itself by very rapid formation of lead compound precipitates, and it has been found that this decomposition of the lead alkyl compound is accompanied by an aggravation of the objectionable corrosiveness that exists when moisture is present. This corrosiveness becomes apparent in the rusting of metal containers for the fuel, since it is difficult to fully exclude moisture, and the aggravation of the corrosive action may be ascribed to the electrolytic action of salts derived from the decomposed anti-knock agent which find their way into the moisture present with the fuel.

An object of this invention is to provide a protection against the undesirable action of sunlight on the organo-metallic compounds, such as lead alkyl compounds.

Another object is to prevent corrosive substances from being incorporated into fuels containing tetraethyl lead.

A further object is to preserve the clarity and stability of refined gasolines containing tetraethyl lead and to confer on the gasoline fuels an inertness to metals of fuel containers.

Objects of the present invention are satisfactorily accomplished by having present with an organo-metallic compound, such as tetraethyl lead, a small amount of a base metal salt of an aromatic sulfide. The preferred base metal constituents of these salts are the alkali and alkaline-earth metals.

The preferred metal salts of aromatic sulfides

are compounds which contain a metal constituent linked to an aromatic nucleus thru oxygen. Analogous compounds suitable for use in the present invention are those in which the metal constituent is attached to the aromatic nucleus thru some other negative radical or negative atom, such as sulfur. Also, in general, it is preferred to have the aromatic nucleus or aryl radical in the compound contain an alkyl side chain substituent, e. g., propyl, isopropyl, butyl, isobutyl, amyl, or isoamyl radicals, or analogous aliphatic radicals in order to obtain the desired degree of solubility in gasoline.

Salts of hydroxy-aromatic sulfides belonging to the class described may be represented by the following type formula:



wherein Ar indicates a substituted aromatic nucleus and M is the metal constituent linked thereto thru oxygen. Analogous compounds have the type formula  $M(XAr)_2(S)$ , wherein X represents, generically, a negative radical or atom.

The characteristic formula may have a number of modifications, for example, the aromatic radical may be mono- or poly-cyclic; the number, kind, and position of alkyl substituents in any of the aromatic nuclei may be varied; also, other substituent groups, e. g., amino groups, alkoxy groups, may be introduced.

The aromatic nuclei in the salts may be united thru a sulfide linkage containing more than one sulfur atom as in  $M(OAr)_2(S)_2$ , but the mono-sulfide linkage is preferred.

The metal salts of the aromatic sulfides may be prepared either by direct reaction of a base metal hydroxide or metal alcoholate with an acidic aromatic sulfide, e. g., a hydroxy aromatic sulfide or aroxy sulfide, if the metal constituent is strongly basic. If the metal is not strongly basic, or if the aromatic sulfide has a very weak acidic function, it is better to replace sodium in a sodium salt of the aromatic sulfide by the desired heavier base metal thru double decomposition with an alcoholic solution of its salt or its alcoholate.

As a specific illustration, the convenient method for preparing the barium salt derivative of an aromatic sulfide is given in the following example:

(Di-isobutyl)-phenol sulfide (442 g.) is dissolved in 3 liters of pure benzene, and 331 grams of barium hydroxide octahydrate  $Ba(OH)_2 \cdot 8H_2O$ , are added. The mixture is refluxed for several hours in a flask fitted with a condenser having a

trap for removal of condensed water. The reaction mixture is filtered and the filter residue added to hot benzene and refiltered. The two filtrates are combined and the solvent removed, yielding the salt bis (barium diisobutyl phenolate) sulfide as a yellowish pulverizable solid. The barium content of the salt was 22-23%.

It is an important advantage of the present invention that the described metal salts can be used in small quantities to accomplish the desired objects. They have been proved to be effective in concentrations ranging from 0.01% to 1% by weight with refined gasolines containing from  $\frac{1}{2}$  to about 3 cc. of tetraethyl lead per gallon for preventing the deterioration of the tetraethyl lead on exposure to actinic light radiations and in counteracting corrosion of iron, steel, and aluminum when the gasoline is wet.

The following data illustrates the efficacy of the described barium salt in a finished aviation gasoline containing 3 cc. of tetraethyl lead per gallon:

TABLE  
*Tests on aviation gasoline containing 3 cc. of tetraethyl lead per gallon*

| Concentration of added barium salt | Effects of sunlight exposure       | Corrosion of steel strip in composition containing added water for 8 days |
|------------------------------------|------------------------------------|---------------------------------------------------------------------------|
| Blank                              | Precipitate in less than 1 hr.     | Severe.                                                                   |
| 0.002%                             | Slight precipitation after 1 day.  | Very slight.                                                              |
| 0.04%                              | Slight precipitation after 8 days. | None.                                                                     |
| 0.8%                               | No precipitation after 8 days.     | Do.                                                                       |

It was observed in carrying out numerous tests with no stabilizing agent present, precipitation of the organo-metallic compound in a refined gasoline begins to occur in less than 1 hour upon exposure to diffused sunlight transmitted thru glass, and likewise the corrosion of metal strips becomes visible in less than 1 hour. With the presence of 0.04% by weight of the barium salt, corrosion was completely suppressed for well beyond 8 days and precipitation was markedly inhibited for a corresponding period. Higher concentrations will completely prevent precipitation on exposure to sunlight.

The compounds used in accordance with the present invention for stabilizing tetraethyl lead or similar organo-metallic compounds are advantageously added to finished gasoline stocks which have been subjected to complete refining so that they satisfactorily pass the A. S. T. M. copper strip corrosion test for fuels, and are practically free of sulfur-containing substances detrimental to the anti-knock effectiveness of tetra-

ethyl lead. The gasoline fuel stock may be derived by cracking, or straight distillation, from liquefied petroleum gases, or from various synthetic reactions. In general, the gasoline should be purified to the extent that it is doctor sweet, contains less than 0.004% reactive sulfur, and shows no copper strip corrosion for 3 hours at 122° F. Compositions containing the stabilized organo-metallic agent may have incorporated other types of blending agents useful for preserving the effectiveness of the organo-metallic compounds or for improving the compositions in which they are employed.

The foregoing discussions and examples are intended to be illustrative only and not to limit the scope of the invention. It is not intended that the invention be limited by any theory, and any modification which conforms to the spirit of the invention is intended to be included within the scope thereof.

I claim:

1. A liquid composition containing tetraethyl lead and a salt of an aromatic sulfide sufficient to increase the stability of the tetraethyl lead to the action of light, such salt having the composition indicated by the formula  $M(XAr)_2(S)$  in which Ar indicates an aromatic nucleus, M is a metallic constituent selected from the class consisting of alkali metals and alkaline earth metals, and X is a negative substituent selected from the class consisting of oxygen and sulfur.

2. A liquid composition containing tetraethyl lead stabilized against decomposition by an alkaline earth metal salt of a hydroxy-aromatic sulfide, said salt having the composition indicated by the formula  $M(XAr)_2(S)$  in which Ar indicates an aromatic nucleus, M is an alkaline earth metal, and X is a negative substituent selected from the class consisting of oxygen and sulfur.

3. A composition comprising tetraethyl lead and bis (barium diisobutyl phenolate) sulfide, to inhibit deterioration of the tetraethyl lead.

4. A composition as described in claim 3, in which the tetraethyl lead and said sulfide are blended with a refined gasoline which is practically free of sulfur-containing substances which are detrimental to the anti-knock effectiveness of tetraethyl lead.

5. The method of protecting a solution of an organo-lead anti-knock agent in gasoline against decomposition by actinic light, which comprises incorporating in the solution a salt of an aromatic sulfide, said salt having the composition indicated by the formula  $M(XAr)_2(S)$  in which Ar indicates an aromatic nucleus, M is a metal selected from the class consisting of alkali metals and alkaline earth metals, and X is a negative substituent.

HARRY W. RUDEL.